

## UNITED STATES PATENT OFFICE

SAMUEL RUBEN, OF NEW ROCHELLE, NEW YORK, ASSIGNEE TO RUBEN CONDENSER COMPANY, OF NEW ROCHELLE, NEW YORK, A CORPORATION OF DELAWARE

METHOD OF MAKING ELECTROLYTIC CONDENSERS AND PREPARING ELECTRODES  
THEREFOR

No Drawing.

Application filed April 12, 1932. Serial No. 604,870.

This invention relates to a method of making electrolytic condensers of the type commonly known as "dry" electrolytic condensers and in preparing the anode member prior 5 to assembly.

A general object of the invention is the provision of such a method which insures the economical, efficient and uniform production of condensers of this type having a low power 10 factor and series resistance, and a degree of mechanical perfection heretofore unattainable uniformly in commercial production.

A more specific object of the invention is the provision of such a method whereby the 15 film-formed anode member is provided with a coating of viscous bonding liquid which insures uniform contact between the film-face of the anode member and the film-maintaining composition or electrolyte, and a low 20 power factor and series resistance.

A further object of the invention is the provision of such a method whereby the film-formed anode member prior to assembly in the condenser is cleaned and then coated with 25 a viscous bonding liquid miscible with the film-maintaining composition and including or consisting of one or more of the polyhydric alcohols or products thereof having two or more hydroxyl radicals which insures efficient 30 electrical contact between the film-maintaining composition and substantially the entire area of the anode member adjacent thereto, uniformity in production and operating characteristics and a very low power factor 35 and series resistance.

Other objects of the invention will in part be obvious and will in part appear herein-after.

The invention accordingly comprises the 40 several steps and the relation of one or more of such steps with respect to each of the others thereof, which will be exemplified in the method hereinafter disclosed, and the scope of the application of which will be 45 indicated in the claims.

Prior to the present invention electrolytic condensers of two types have been used, the gas layer polarized cell type and the electrolytically formed film layer type. The electrolytic condensers made by the method of

the present invention are of the latter type. Such condensers are composed fundamentally of a pair of electrodes, preferably in the form of sheets or plates, at least one of which is formed from a suitable valve metal, such 55 as, for example, aluminum, tantalum, magnesium or alloys thereof, provided with an electrolytically formed current-blocking film. Between these electrodes is disposed a body or layer of a viscous composition 60 of paste consistency which may be spread on suitable spacer material used as a separator for the electrodes. In its usual form this composition comprises a vehicle in which is suspended a suitable film-forming 65 electrolyte. This vehicle is usually a polyhydric alcohol having two or more hydroxyl radicals, for example, a glycol or a glycerol.

When such condensers are used in power filter circuits where efficiency and high capacitances are essential, those known to the prior art have been found to have certain undesirable limitations. The resistance of the electrolyte or film-maintaining composition being relatively high gives a relatively high 75 series resistance to such condensers, resulting in relatively high heat losses and a high power factor. Furthermore, in commercial production it has been found that the effective area of the film-formed anode member is considerably reduced by separation 80 between the film-maintaining composition or electrolyte and the anode member. This is more frequently experienced in the coil type wherein the electrodes are wound up with 85 spacer material spread with film-maintaining composition interposed between the electrodes. In the so-called "dry" electrolytic condensers wherein the film-maintaining 90 composition or electrolyte is of paste consistency there is usually found a somewhat granular structure which has a relatively low surface flexibility. Areas of separation thus appear when thin layers thereof are deformed. In addition these difficulties make 95 uniformity in commercial production difficult.

By the present invention an economical method of making such electrolytic condensers and preparing the anode member 100

thereof is provided, which substantially eliminates these difficulties of the prior art and which is particularly adapted for the improvement of electrolytic condensers comprising aluminum electrodes, one of which is provided with a current-blocking film preferably separated by spacer material upon which is spread a composition including a glycol or glycerol, preferably ethylene glycol, and a film-maintaining electrolyte, preferably ammonium borate and boric acid.

The method of the present invention comprises coating the film-formed electrode with a viscous bonding liquid miscible with the film-maintaining composition prior to assembly in the condenser unit. Any practicable method of applying such a coating to a film-formed electrode may be used in accordance with the present invention. The preferred method, however, is as follows: The metal electrode, preferably in the form of a sheet, is electrolytically treated in a suitable electrolyte so as to have formed on it a current-blocking film, and is then cleaned, preferably by passing the film-formed sheet successively through a bath of alcohol and a bath of water, distilled water being preferred to prevent undue contamination. The cleaned film-formed sheet is then preferably passed through or dipped into the chosen viscous bonding liquid to provide a thin coating thereof on the film-formed electrode sheet. Spacer material is then placed on the sheet and spread with a layer of suitable film-maintaining composition preferably viscous and of plastic consistency and of a less degree of fluidity than the viscous bonding liquid, so that the coating of bonding liquid makes intimate contact with the film-maintaining composition. A second electrode plate, the cathode, is then laid over the spacer material and film-maintaining composition, the latter being compressed between the two electrodes to insure good physical contact between the anode, the viscous bonding liquid, the film-maintaining composition and the cathode. If the condenser is to be rolled, another layer of spacer material is then placed over the cathode, spread with film-maintaining composition, and the rolling carried out in the usual manner.

The viscous bonding liquid may consist of or include one or more of the polyhydric alcohols or products thereof having two or more hydroxyl radicals, such as, for example, glycerine, ethylene glycol, glucoses, etc. The preferred polyhydric alcohols are those falling within the classes glycols and glycerols.

In the specification and claims the term "viscous bonding liquid" is intended to cover any liquid, viscous in consistency, comprising one or more ingredients of greater fluidity than the film-maintaining composition and which is readily miscible with the latter and electrically-conductive in the completed

condensers; the term "film-formed electrode" is used to designate an electrode of suitable valve metal provided with a current-blocking film; and the term "film-maintaining composition" is used to designate any composition used in the final assembly including a film-maintaining electrolyte for the purpose of maintaining a current-blocking film on the electrode.

While I do not wish to limit myself to any particular theory it is believed that the coating of viscous bonding liquid on the film-formed electrode serves as a protection for the current-blocking film thereon and in addition provides a flexible electrical bond between the film-maintaining composition and the current-blocking film of the electrode insuring electrical contact therebetween substantially throughout the entire area of the film-formed electrode over which the film-maintaining composition lies. It serves to bring the electrical charge from the cathode through the film-maintaining composition to the current-blocking film on the anode and thus provides maximum capacitance per unit of electrode area and reduces the series resistance and the power factor of the condenser unit to a minimum. For example, tests have shown that prior to the present invention condensers comprising aluminum electrodes and a film-maintaining composition of ammonium borate, boric acid and ethylene glycol having a capacity of 10 mfd., under the best conditions have a resistance of about 3 to 4 ohms. Similar condensers made in accordance with the method of the present invention, that is, by providing the anodes with a coating of viscous bonding liquid prior to the application of the spacer material and film-maintaining composition, have been found to have a resistance of around 1 ohm. The average power factor of the latter units has been found to be better than one per cent as compared with a power factor of about 3 to 4 per cent for the former units and a surprising uniformity in these units has been attained in commercial production.

It will thus be seen that in accordance with the present invention a method for making electrolytic condensers and preparing electrodes therefor has been provided which efficiently attains the objects set forth above. The characteristics of electrolytic condensers made in accordance with the present invention indicate an efficiency in operation and possible fields of use, such as, for example, in alternating current work and more particularly in motor starting, due to the extremely small resistance loss, heretofore unattainable with the best condensers of this type available prior to the present invention.

Since certain changes may be made in carrying out the above method without departing from the scope of the invention, it is in-

tended that all matter contained in the above description shall be interpreted as illustrative and not in a limiting sense.

It is also to be understood that the following claims are intended to cover all of the generic and specific features of the invention herein described, and all statements of the scope of the invention which, as a matter of language, might be said to fall therebetween.

10 Having described my invention, what I claim as new and desire to secure by Letters Patent, is:

1. The method of preparing electrodes for electrolytic condensers of the so-called "dry" type having a film-maintaining composition of at least paste consistency comprising applying a coating of viscous bonding liquid to electrode metal provided with a current-blocking film, said coating being adapted to 15 form a bond between the current-blocking film and the paste-like film-maintaining composition when the elements of the condenser are assembled.

2. The method of preparing electrodes for electrolytic condensers of the so-called "dry" type having a film-maintaining composition of at least paste consistency comprising cleaning film-formed electrode metal and applying thereto a coating of viscous bonding 20 liquid, said coating being adapted to form a bond between said film-formed electrode and the paste-like film-maintaining composition when the elements of the condenser are assembled.

3. The method of preparing electrodes for electrolytic condensers of the so-called "dry" type having a film-maintaining composition of at least paste consistency comprising applying a coating of viscous bonding liquid 30 including one or more of the polyhydric alcohols or products thereof having two or more hydroxyl radicals to electrode metal provided with a current-blocking film, said coating being adapted to form a bond between the current-blocking film and the paste-like film-maintaining composition when the elements of the condenser are assembled.

4. The method of preparing electrodes for electrolytic condensers of the so-called "dry" type having a film-maintaining composition of at least paste consistency comprising applying a coating of viscous bonding liquid including a polyhydric alcohol falling within the classes glycols and glycerols to an 40 aluminum member provided with a current-blocking film, said coating being adapted to form a bond between the current-blocking film and the paste-like film-maintaining composition when the elements of the condenser are assembled.

5. The method of preparing electrodes for electrolytic condensers of the so-called "dry" type having a film-maintaining composition of at least paste consistency comprising 45 cleaning a film-formed aluminum member

and applying thereto a coating of viscous bonding liquid including a polyhydric alcohol falling within the classes glycols and glycerols, said coating being adapted to form a bond between said film-formed electrode and the paste-like film-maintaining composition when the elements of the condenser are assembled.

6. The method of preparing electrodes for electrolytic condensers of the so-called "dry" type having a film-maintaining composition of at least paste consistency comprising passing a film-formed aluminum member through a bath of ethylene glycol, to provide thereon a coating adapted to form a bond between said film-formed electrode and the paste-like film-maintaining composition when the elements of the condenser are assembled.

7. The method of preparing electrodes for electrolytic condensers of the so-called "dry" type having a film-maintaining composition of at least paste consistency comprising passing a film-formed aluminum member successively through baths of alcohol, water and ethylene glycol, to clean said film-formed aluminum member and subsequently to provide thereon a coating adapted to form a bond between said member and the paste-like film-maintaining composition when the elements of the condenser are assembled.

8. The method of preparing electrodes for electrolytic condensers of the so-called "dry" type having a film-maintaining composition of at least paste consistency comprising applying a coating of viscous bonding liquid of greater fluidity than the film-maintaining composition with which it is miscible to electrode metal provided with a current-blocking film, said coating being adapted to form a bond between the current-blocking film and the paste-like film-maintaining composition when the elements of the condenser are assembled.

9. The method of making electrolytic condensers which consists in cleaning a film-formed anode, applying a coating of viscous bonding liquid to said anode, applying a film-forming composition of paste consistency thereto and bringing a second electrode member into physical contact with said composition.

10. The method of making electrolytic condensers which consists in providing an aluminum sheet anode member with a current-blocking film, cleaning said film-formed anode member, coating said anode member with a viscous bonding liquid including one or more of the polyhydric alcohols or products thereof having two or more hydroxyl radicals applying to the said coated anode a film-forming composition of paste consistency and bringing a second electrode member into physical contact with said composition.

11. The method of making electrolytic condensers which consists in providing an alumini-

num sheet anode with a current-blocking film, passing said film-formed anode member successively through baths of alcohol, water, and a viscous bonding liquid including one or 5 more of the polyhydric alcohols or products thereof having two or more hydroxyl radicals applying to said anode member a film-forming composition of paste consistency, and bringing a second electrode member into 10 physical contact with said composition.

12. The method of making electrolytic condensers which consists in providing an aluminum sheet anode member with a current-blocking film, passing said film-formed anode 15 member successively through baths of alcohol, water and ethylene glycol and positioning said anode member adjacent to another electrode member spaced therefrom by spacer material and a film-forming composition of 20 paste consistency including ammonium borate, boric acid and ethylene glycol.

13. The method of making electrolytic condensers which consists in passing sheet aluminum successively through a film-forming electrolyte, a bath of alcohol, a bath of 25 water and ethylene glycol and winding up into coil form said treated aluminum sheet with another sheet of metal having a strip of spacer material on each face thereof provided with a composition of paste consistency 30 including ammonium borate, boric acid and ethylene glycol.

In testimony whereof I affix my signature.  
SAMUEL RUBEN.

25

40

45

50

55

60

65